

Jan. 22, 1924.

1,481,761

F. THARALDSEN

PROCESS FOR ELECTROTHERMIC PRODUCTION OF ZINC

Filed May 25, 1922

*Fig. 2.*



*Fig. 1.*



Inventor

*Felix Tharaldsen.*

By

*B. Anger,*

Attorney

Patented Jan. 22, 1924.

1,481,761

# UNITED STATES PATENT OFFICE.

FILIP THARALDSEN, OF CHRISTIANIA, NORWAY.

## PROCESS FOR ELECTROTHERMIC PRODUCTION OF ZINC.

Application filed May 25, 1922. Serial No. 562,612.

To all whom it may concern:

Be it known that I, FILIP THARALDSEN, a citizen of Norway, residing at Christiania, Norway, have invented certain new and useful Improvements in Processes for Electrothermic Production of Zinc, for which I have filed application for patent in Norway June 27, 1918, and of which the following is a specification.

10 The object of the invention is to provide an improved process of production of zinc in electric resistance furnaces.

In the electrothermic production of zinc in resistance furnaces it has been proposed 15 to arrange the charge consisting of zinc-bearing materials and reducing agents as an even horizontal layer on a stratum of coke, which latter serves as heating resistance. In this way a very uniform transfer 20 of heat to the charge is secured, and the electric efficiency of the furnace is very high. The layer of coke serves as heating resistance and at the same time it prevents the charge from getting in immediate contact 25 with the bottom of the furnace and sticking to it in baking.

According to the present invention the zinc containing charge proper is used as heating resistance. By convenient composition 30 of the charge it has proved possible to obtain sufficient conductivity in the charge and also to prevent molten slag from getting in touch with the hearth of the furnace. Generally speaking the invention can 35 be carried out by using a sufficient surplus of reducing agent in the charge. However the invention more specially aims at using pure or nearly pure oxide of zinc as raw material. A charge consisting of zinc oxide 40 and reducing agent has proved serviceable as heating resistance even without containing any considerable surplus of reductive and the detrimental effect of molten slag upon the bottom of the furnace does not 45 make itself felt as in this case such masses are not formed to any appreciable extent, the whole charge being volatilized except a trifling residue of excess carbon, which however does no harm.

50 A charge of zinc oxide and carbon has a very considerable conductivity owing to the finely divided state of the oxide and because of the absence of rocky constituents.

In order to secure a uniform heating of 55 the charge notwithstanding that its conductivity is greater in the hot state than when

relatively cold, the invention provides a pre-heating of the charge before it arrives in the zone of the furnace, where the resistance heating occurs. This preheating is effected for instance in the manner, that the charge, which is introduced into the furnace in the shape of a uniform thin layer, is first exposed to radiation from an electric arc, and then when it has assumed a convenient temperature and conductivity it is subjected to direct passage of the current.

The type of furnace used for carrying out the invention is shown on the accompanying drawings in which—

Figure 1 is a transverse section on the plane indicated by the line 1—1 of Figure 2.

Figure 2 is a longitudinal section on the plane indicated by the line 2—2 of Figure 1.

The furnace has a movable hearth on which a charge is placed outside the furnace chamber, and said hearth conveys the charge into the furnace, thereby distributing the charge in the form of a horizontal layer, which is subjected to reduction successively as it advances through the furnace chamber.

The arrangement of the charge as a horizontal layer is of special importance, because it secures one and the same section for the passage of the electric current and consequently a uniform resistance. The heating of the charge is then uniform all over the hearth.

In the furnace shown in the drawing the electric current is supplied by means of the electrodes A. to the uniformly distributed charge B. on the hearth C. The movement of the hearth is supposed to be from the left to the right. The preheating of the charge is effected by means of an electric arc between the electrodes D. The zinc vapors evolved in the furnace chamber escape through the outlet E.

Having now fully described my invention and the manner in which it is performed, I hereby declare that what I claim is:

1. The process of electrothermically producing zinc consisting in first heating a charge of zinc oxide and carbon by radiation from an electric arc, and then subjecting the charge to the direct passage of the electric current therethrough.

2. The process of electrothermically producing zinc consisting in first preparing a charge of zinc oxide and carbon in a layer

of uniform thickness and substantially uniform electrical resistance at all points, heating such charge by radiation from an electric arc, and then subjecting the charge to the direct passage of the electric current therethrough.

3. The process of electrothermically producing zinc consisting in first preparing a charge of zinc oxide and carbon in a layer 10 of uniform thickness and substantially uniform electrical resistance at all points, mov-

ing such charge through a furnace, and heating such charge while moving, first by radiation from an electric arc, and then subjecting such charge to the direct passage of 15 the electric current therethrough.

In testimony whereof I affix my signature in presence of two witnesses.

FILIP THARALDSEN.

Witnesses:

P. BRODAE,  
H. FURTNASS.